

# UNITED STATES PATENT OFFICE.

WILLIAM AUGUSTUS HALL, OF NEW YORK, N. Y., ASSIGNOR TO AMERICAN MAHOGANY COMPANY, A CORPORATION OF MAINE.

## ART OF COLORING AND FIREPROOFING WOOD.

961,123.

Specification of Letters Patent. Patented June 14, 1910.

No Drawing.

Application filed June 6, 1908. Serial No. 437,078.

To all whom it may concern:

Be it known that I, WILLIAM A. HALL, a citizen of the United States, residing at New York, in the county of New York and State of New York, have invented or discovered certain new and useful Improvements in the Art of Coloring and Fireproofing Wood, of which the following is a specification.

This invention relates to the art of transforming wood by coloring and fireproofing the same, so as to produce, from the cheaper or more common varieties of wood, such as birch, maple or gumwood, close fireproofed imitations of rarer or more expensive woods, such as black walnut, mahogany, etc.

The object of the invention is accomplished by a novel method of treating the inexpensive woods so as to render them fireproof and give them the appearance and texture throughout their bodies of the more costly woods.

The invention is carried into effect by causing suitable coloring and fireproofing solutions to permeate the wood and to be diffused throughout its body so that when the wood is cut up, in making cabinet work, or for other purposes, all parts of it will be suitably colored and will be of a fireproof character, and there will be practically no uncolored, non-fireproofed streaks in the wood, but the coloring and fireproofing materials will be infused and diffused throughout the wood, but with considerably more of the coloring matter deposited in the softer or more porous portions of the wood, such as the annual rings and open grain vessels, thereby resulting in a very prominent development of the "grain" or figure of the wood.

The invention may be carried into effect either by what is known as the vacuum and pressure process, or by what may be referred to as the open vat treatment.

In practicing the invention by the vacuum and pressure process well-dried lumber, in the shape of boards, planks, flitches or deals, of any convenient size, is subjected, in a closed receptacle, to a vacuum action sufficiently powerful and continued sufficiently long to remove from the wood practically all the air therein contained, so as to make it absorbent or receptive to the fluids to be applied later. It has been found preferable, during the vacuum process, to subject the wood to a moderate heat of say from 90° to

100° F., which has a tendency to open the pores of the wood. A combined coloring and fireproofing solution is then drawn or pumped into the receptacle or chamber containing the wood until the wood is fully immersed in such solution. The coloring and fireproofing solution may be applied either hot or cold (preferably the former) according to its characteristics, and the solution will be rapidly taken up by the absorbent wood. When the receptacle is filled with the solution, hydraulic or pneumatic pressure, preferably of say 200 to 300 pounds or more to the square inch, is applied to the chamber of the receptacle and is maintained until the wood is impregnated by the coloring and fireproofing solution to as great a degree as possible; the time required for this varying from two to three hours to ten or twelve hours or more, according to the thickness or hardness of the lumber under treatment and the amount of pressure maintained.

The coloring solutions used may be of any character that have a sufficiently high capillary activity, but alkaline aqueous solutions of bark or wood extract, such as those produced from hemlock, spruce or mahogany, are preferred, the coloring materials selected of course being those which will not be injured to any extent by temperatures of 212° F., or thereabout.

The fireproofing solutions which are to be mixed with the alkaline coloring solutions, must be of such a character as not to precipitate the coloring solutions, and the coloring solutions must be of such a character as not to injure or deteriorate the fireproofing solutions in any way, by reason of being antagonistic thereto. The fireproofing composition which I have found, by extended experiments, to be most satisfactory consists of a mixture of sulfate of ammonia and phosphate of soda. Sulfate of ammonia is a very strong fireproofing substance which not only mineralizes the fiber of the wood, but, which when subjected to heat, discharges ammonia gas which has a tendency to extinguish flame. Owing, however, to the acid character of this salt it is not suitable for use alone with alkaline coloring solutions, as it has a tendency to precipitate such solutions, so that they can not be made to permeate the wood as thoroughly as may be desired. Also this acid salt cannot be used

alone as a fireproofing substance in connection with alkaline coloring solutions, for the reason that the fireproofing qualities of the fireproofing substance are greatly impaired or destroyed by such alkaline solutions. But 5 I have discovered that by mixing a suitable proportion of phosphate of soda, which is an alkaline fireproofing salt, with the sulfate of ammonia the acid of the latter is neutralized and the whole mixture is rendered 10 neutral or slightly alkaline; and such fireproofing mixture will not precipitate or injure the alkaline coloring solutions or substances with which it may be mixed, nor 15 will the fireproofing qualities of the mixture be impaired by the alkaline solution. While phosphate of soda is not, of itself, so strong a fireproofing substance as sulfate of ammonia, I have found that a mixture of these 20 two salts is more strongly fireproofing than either when used alone, for the reason that the sulfate of ammonia is not, of itself, a very good mineralizing salt, its fireproofing qualities being largely due to the evolution 25 of gases which do not support combustion; whereas the phosphate of soda is a very strong mineralizer, but is deficient in a capability of evolving flame-extinguishing gases. While the invention is not to be understood as being limited to any particular 30 proportions of these fireproofing salts in the mixture, it may be stated that experiments have determined that phosphate of soda may, and preferably will, form from one-third to one half of the mixture.

35 Instead of using sulfate of ammonia in the fireproofing mixture, phosphate of ammonia might be used with equally good effect; but owing to the much greater cost of the latter salt the former will preferably be employed. Also, instead of using phosphate 40 of soda as an alkaline substance in the fireproofing mixture sulfid of soda might be employed; but the former salt is much preferred owing to its greater efficiency. Other 45 fireproofing substances or solutions which, either alone or when combined together will be of a neutral or alkaline character, or which will not be deteriorative of or injurious to the coloring solutions, may also be used in place of the preferred salts or substances above mentioned; and the invention or discovery is therefore not to be understood as being limited to any particular fireproofing substances so long as those employed form a composition which is of a neutral or alkaline character and which is harmonious with or non-antagonistic to the alkaline coloring solutions.

55 60 Instead of effecting the coloring and fireproofing of the wood by the vacuum and pressure process above described, well-dried wood may be immersed in a coloring and fireproofing solution, of the character hereinbefore indicated, contained in an open vat

or receptacle, and in which it may be boiled for two or more days, to cause the coloring and fireproofing solutions to permeate the wood and to be properly diffused therein; or, instead of being boiled in a combined 70 coloring and fireproofing solution the wood may first be boiled in the coloring solution in an open vat and afterward plunged into a cold fireproofing solution which, owing to contraction, will be caused to be absorbed 75 by or struck into the wood; and this cold fireproofing solution may afterward be heated, and by boiling the wood therein for some time the coloring and fireproofing materials will be thoroughly diffused throughout the wood.

It will be understood that wood which has been subjected to a coloring and fireproofing treatment by either of the methods above described will be so transformed as to 85 closely resemble the higher priced wood which it may be desired to imitate, according to the character of the coloring solutions which may be employed in this treatment; and such wood will also be rendered fireproof. The treatment of the wood by either of the methods above described has a tendency to harden and toughen the wood, and also serves greatly to develop the grain 90 thereof, so that natural woods having but 95 little grain figure will come out with a highly developed and beautifully figured "grain", and will therefore be very desirable for any purpose where an ornamental fireproofed wood may be employed. This 100 result is largely due to pigment-like deposits of the coloring matters in the grain cells, together with the fireproofing salts, such deposits resulting from precipitation of the coloring matters from the coloring solutions 105 partly by dialyzation and partly by the effect of the weak natural acids contained in the wood.

Having thus described my invention I claim and desire to secure by Letters Patent: 110

1. The herein described fireproofed and artificially colored wood, having harmonious coloring and fireproofing materials distributed and diffused together throughout the wood, and the "grain" of the wood highly 115 developed.

2. The herein described fireproofed and artificially colored wood, having an artificial coloring material and a mixture of acid and alkaline fireproofing salts distributed and diffused throughout the same, and the "grain" of the wood highly 120 developed.

3. The herein described fireproofed and artificially colored wood, having an artificial coloring material and a mixture of sulfate of ammonia and phosphate of soda distributed and diffused throughout the same, and the "grain" of the wood highly 125 developed.

4. The herein described process for color- 130

ing and fireproofing wood, consisting in infusing coloring and fireproofing materials into and throughout the wood simultaneously, the coloring solution being of an alkaline character, and the fireproofing material consisting of a mixture of acid and alkaline salts.

5. The herein described process for coloring and fireproofing wood, consisting in infusing coloring and fireproofing materials into and throughout the wood simultaneously,

ously, the coloring solution being of an alkaline character, and the fireproofing material consisting of a mixture of sulfate of ammonia and phosphate of soda.

15

In testimony whereof I affix my signature, in presence of two witnesses.

WILLIAM AUGUSTUS HALL.

Witnesses:

JOHN CARRINGTON YATES,  
WALTER M. SCHEUMAKER.